

# United States Patent [19]

Falivene

[11]

4,057,673

[45]

Nov. 8, 1977

[54] FABRIC CONDITIONING WITH IMPROVED COMPOSITION CONTAINING A PLASTICIZER

[75] Inventor: Pasquale J. Falivene, Union City, N.J.

[73] Assignee: Colgate Palmolive Company, New York, N.Y.

[21] Appl. No.: 630,605

[22] Filed: Nov. 10, 1975

## Related U.S. Application Data

[63] Continuation of Ser. No. 513,238, Oct. 9, 1974, abandoned, which is a continuation of Ser. No. 359,395, May 11, 1973, abandoned, which is a continuation of Ser. No. 82,461, Oct. 20, 1970, abandoned.

[51] Int. Cl.<sup>2</sup> ..... B32B 5/16; B05D 3/12

[52] U.S. Cl. ..... 428/411; 427/242; 428/315; 428/407

[58] Field of Search ..... 428/274, 310, 315, 262, 428/279, 411, 407; 427/242

## References Cited

### U.S. PATENT DOCUMENTS

|           |        |                   |               |
|-----------|--------|-------------------|---------------|
| 1,968,795 | 7/1934 | Bertsch           | ..... 252/1   |
| 2,213,477 | 9/1940 | Steindorff et al. | ..... 260/613 |
| 2,936,251 | 5/1960 | Garceau et al.    | ..... 428/375 |
| 3,036,130 | 5/1962 | Jackson et al.    | ..... 260/584 |

|           |         |              |               |
|-----------|---------|--------------|---------------|
| 3,351,483 | 11/1967 | Miner et al. | ..... 252/8.5 |
| 3,442,692 | 5/1969  | Gaizer       | ..... 427/242 |
| 3,501,335 | 3/1970  | Cahn et al.  | ..... 252/8.8 |
| 3,554,784 | 1/1971  | Lyness       | ..... 252/8.8 |
| 3,686,025 | 8/1972  | Morton       | ..... 428/274 |
| 3,743,534 | 7/1973  | Zamora       | ..... 427/242 |

Primary Examiner—William J. Van Balen  
Attorney, Agent, or Firm—Norman Blumenkopf;  
Herbert S. Sylvester; Murray M. Grill

## [57] ABSTRACT

The conditioning of fabrics is effected by compositions which comprise a major proportion of conditioning agent and a minor proportion of a plasticizer. The conditioning agent is preferably a surface active fabric softener and the plasticizer is preferably a water soluble liquid, nonionic poly-lower alkoxy or polyhydroxy compound, which improves the transferability of the conditioning agent to fibrous materials during treatment of such materials, by preventing cracking or flaking of the conditioning agent during the treating operation.

Although in some instances the conditioning agent plus plasticizer composition may be used as a solid product alone, without a separate base, it is generally preferred that it be employed as a coating on a base, preferably a form-retaining solid base. Also, it is preferred that the fabric conditioning be practiced on damp laundry in an automatic laundry dryer.

2 Claims, 9 Drawing Figures





Fig. 1.



Fig. 2.



Fig. 3.



Fig. 4.



Fig. 5.



Fig. 6.



Fig. 7.



Fig. 8.



Fig. 9.

## FABRIC CONDITIONING WITH IMPROVED COMPOSITION CONTAINING A PLASTICIZER

This is a continuation, of application Ser. No. 513,238 filed Oct. 9, 1974, which in turn is a continuation of Ser. No. 359,395, filed May 11, 1973, which is a continuation of Ser. No. 82,461 filed Oct. 20, 1970, each abandoned.

### SUBJECT OF THE INVENTION

This invention relates to the conditioning of fabrics. More particularly, it relates to the employment of a fabric softening and/or antistatic agent with a plasticizer. The plasticizer improves the even transfer of the conditioning agent to the fibrous materials being treated by preventing cracking or flaking off of the conditioning agent at the surface of a conditioning article.

### BACKGROUND OF THE INVENTION

In the conditioning of fabrics, such as those in laundry, by tumbling contact of the laundry with a fabric conditioning article, such as a base material containing a coating of conditioning composition, stains and spots have been observed on the treated articles. In some cases, as when cationic conditioning agents, such as 20 quaternary ammonium salts, are employed, staining may be due to a chemical reaction between color bodies or metal ions and the quaternary compound. However, in addition to such staining, spotting has been observed on items of laundry treated in an automatic dryer with 25 conditioning compositions that were transferred to the laundry from the surfaces of a solid treating article. Such spotting, while unobjectionable in certain cases, sometimes is sufficiently pronounced that it significantly adversely affects the appearance and utility of 30 the conditioned article. This is especially true when the materials being conditioned are resin-coated or otherwise treated to make them "permanently pressed". Because most of the fabric conditioning agents of the type described herein are wax-like the waxy or fatty appearing spots on the laundry will be more apparent on colored items than on white goods, since they seem to 35 deepen the colors. Nevertheless, upon ironing, in which the deposited conditioning agent is usually fused and distributed in a smooth film at the surface of the article 40 being ironed, the spot may be enlarged or may be made readily visible and hence, more objectionable, even on white goods. In some cases ironing may "fix" the stain to the substrate.

Chemical analyses of the substances of the spots on the conditioned fabrics establish that they usually correspond substantially to the conditioning compositions being employed. Thus, it would be natural to assume that under the heat of the conditioning operation, usually undertaken in an automatic laundry dryer, the conditioning composition had melted at the surface of the conditioning article and had been smeared onto the fabric contacting it, creating the spots. Consequently, from such an analysis of the problem it would appear that what was required was a hardening agent for the conditioning composition or else, to employ conditioning agents of higher melting or softening points. Also, in the event that the smearing was due to the softening of the conditioning agent in contact with moisture in laundry being treated, it appeared desirable to utilize conditioning agents of lesser degree of water solubility. From these considerations, the employment of a water soluble, liquid plasticizing compound to diminish spotting

was contraindicated. Even if plasticizers were considered as being of possible utility to make the conditioning composition more uniform and resilient and to aid in the spreading of the conditioning agent over the fabric with which it is brought in contact, it would be expected that the use of liquid and water soluble material would be avoided, in the interest of diminishing the excessive smearing of the conditioning agent onto the fabric being treated.

### DESCRIPTION OF THE INVENTION

Despite the contraindications from the prior art and a reasonable analysis of the problem, it has now been found that the addition to fabric softeners and antistatic agents of a plasticizing agent, generally in minor proportion, improves the uniformity of transfer of such conditioning agents to fabric being treated by tumbling contact with a solid conditioning article under usual automatic laundry dryer conditions of heat and moisture. It seems that the major problems confronted were in the breaking away or flaking off of pieces of conditioning material from the surface of a conditioning article and subsequent fusion of the conditioner pieces onto the material being treated. The use of a liquid plasticizer has significantly improved the surface characteristics of the conditioning composition and has prevented such breaking away of flakes or pieces of conditioning agent, without objectionably softening the conditioning composition to the point where it fuses onto the fabric in lumps or smears which would create spots.

In accordance with the present invention there is provided a solid state composition for use in conditioning fibrous materials to make them soft and/or static-free which comprises a surface active conditioning agent, of either nonionic, anionic or cationic type, plus a plasticizing agent, present in sufficient quantity to improve the transferability of conditioning agent to fibrous material during treatment of the fibrous material with the conditioning composition in an automatic laundry dryer. Transferability is improved by the plasticizer preventing cracking or flaking off of the fabric conditioner during tumbling contact of the material to be conditioned with the solid state conditioning agent. Also within the invention are an article for conditioning fibrous materials which comprises a solid state composition of the type mentioned on a solid base, preferably of the form-retaining type and a method of conditioning fibrous materials utilizing such compositions and articles.

In preferred embodiments of the invention, the conditioning agents employed are nonionic or anionic, the plasticizing agent is a liquid, nonionic poly-lower alkyl or polyhydroxy compound, it is present in a minor proportion, from 1 to 25% of the conditioning composition and conditioning is of damp laundry in an automatic laundry dryer of the tumbling drum type.

Various objects, details, constructions, operations, uses and advantages of the invention, in its various aspects, will be apparent from the following description, taken in conjunction with the illustrative drawing of some embodiments thereof, in which drawing:

### THE DRAWING

FIG. 1 is a top plan view of a fabric conditioning article coated with fabric conditioning composition;

FIG. 2 is a central vertical sectional view along plane 2-2 of the article of FIG. 1, showing the coating composition on a polystyrene foam base;

FIG. 3 is a top plan view of a coated paper conditioning article;

FIG. 4 is a top plan of the article of FIG. 1, without plasticizer in the conditioning composition, after being subjected to automatic dryer conditions, illustrating the flaking off of particles of coating conditioning composition therefrom;

FIG. 5 is a top plan view of an article of FIG. 3, after subjection to dryer conditions, illustrating the flaking off of unplasticized conditioning composition therefrom;

FIG. 6 is a perspective view of the article of FIG. 5, illustrating the bending thereof which promotes removal of unplasticized conditioning composition;

FIG. 7 is a view of a portion of conditioned fabric, 15 showing the deposit thereon of a flake of unplasticized conditioning material;

FIG. 8 is a view of the fabric of FIG. 7, after melting and partial spreading of the unplasticized conditioning composition, due to subjection to the heat of an automatic dryer; and

FIG. 9 is a view of the same fabric, after ironing of the portion thereof containing a deposit of unplasticized conditioning composition.

#### DETAILED DESCRIPTION OF THE INVENTION

Spherical fabric conditioning article 11, shown in FIG. 1, comprises a form-retaining polystyrene foam base 15 coated with fabric softening and antistatic composition 13. As will be noted from FIGS. 1 and 2, the coating is smooth and continuous over the surface of the polystyrene sphere 15 and penetrates below said surface, as illustrated at 17, to better hold the coating to it. In FIG. 3 is shown a similar fabric conditioning article, in which the conditioning composition 19 is deposited on both sides of a paper base 21. FIGS. 1-3 represent both the articles and compositions of the present invention, containing a plasticizing ingredient, and also, when the plasticizer is omitted from the coating, repre- 40 sent control articles.

In FIG. 4, the coating 13 of conditioning composition is one not containing plasticizer. Accordingly, during subjection of the spherical conditioning article to the automatic laundry dryer conditions, wherein it is contacted against the metal interior walls of a dryer and flights thereon, sections of coating are removed as flakes, leaving voids 23. Similar voids 25 are shown on conditioning article 27 of FIG. 5. The bending which strains unplasticized coating composition 21 so as to 50 cause the flaking off of coating composition and the creation of voids, such as that at 25, is illustrated in FIG. 6. Such bending may be caused by entrapment of a flexible article between items of laundry.

In FIG. 7 is shown a piece of laundry or fabric 29 on which there has been undesirably deposited a flake 31 of unplasticized conditioning material, which had been removed from the conditioning article during a treating operation. The same fabric, with the deposit 33 having been fused into the fabric over a larger area by dryer operation is illustrated in FIG. 8. Similarly, a further enlarged spot 35 is apparent after ironing of article 29.

Although it is within the broad contemplation of the present invention that fabric conditioning compositions are improved by the incorporation therein of plasticizers and are then better usable for the treatment of textiles to soften them, make them antistatic or give them other desirable properties, usually such compositions

will be most beneficial when employed on a conditioning article as a coating on a base or substrate, preferably one of form-retaining material. When they are used as coatings on flexible bases, such as paper or cloth, the advantage of the plasticizer content is most significant, because of the bending and folding such materials normally encounter in use, with the resultant strains on unplasticized conditioning coatings that tend to make them crack or flake off onto the fabrics being treated.

Of the form-retaining bases that are coated, it will be preferred to employ those which are of low densities, such that the calculated density will be on the order of from 0.1 to 2 grams/cubic centimeter, preferably from 0.2 to 0.5 g./c. cm. Such materials include various woods, composition boards, paperboards, light minerals, rubbers and synthetic organic polymeric plastics, preferably foamed plastics such as polyurethanes, polyesters, polystyrenes, polyvinyl chlorides or nylons. Such items may be formed by various means including folding, molding, cementing, fusing, stapling and interlocking of parts to make the final desired shape. Normally, to diminish strains on the coating agent, sharp corners will be avoided on the base to be coated. Instead of using form-retaining materials, flexible substrates, such as sheet materials of paper, cloth, sponge, rubber, synthetic organic polymeric plastics and similar materials may be used. These will also generally be light in weight and will usually be of thicknesses from 0.001 to 1 cm., preferably from 0.003 cm. to 0.1 cm. The volumes of the form-retaining articles will normally be from 5 to 500 c. cm., preferably from about 10 to 100 c. cm., while the sizes of the sheet materials or flexible substrates will usually be from 50 sq. cm. to 2,000 sq. cm., preferably from 100 sq. cm. to 1,000 sq. cm.

Among the fabric softeners and antistatic agents that are usable in accord with the present invention are the nonionic surface active materials, including higher fatty acid mono-lower alkanolamides, higher fatty acid di-lower alkanolamides, block copolymers of ethylene oxide and propylene oxide, having hydrophilic and lipophilic groups, alkyl (preferably middle alkyl) phenol poly-lower alkylene oxide lower alkanols, polymers of lower alkylene glycols, polyalkylene glycol ethers of higher fatty alcohols and polyalkylene glycol esters of higher fatty acids. Among the anionic agents are the higher fatty acid soaps of water soluble bases, higher fatty alcohol sulfates, higher fatty acid monoglyceride sulfates, sarcosides, taurides, isethionates and linear higher alkyl aryl sulfonates. Cationic compounds include the higher alkyl di-lower alkyl amines, di-higher alkyl lower alkyl amines and quaternary compounds, especially quaternary ammonium salts, e.g., quaternary ammonium halides. In the preceding description, lower, as applied to various hydrocarbyl-containing groups, indicates a carbon content of from 1 to 6, preferably from 2 to 3. Similarly, higher includes compounds having from 10 to 20 carbon atoms, preferably from 12 to 18. Of course, since it is important to the present invention that the conditioning composition be in a solid form, so that it can have conditioning agent gradually removed from it by contact with tumbling laundry fabrics in a dryer or similar machine, the fabric softening and/or antistatic agents will be chosen to be in the solid state. Nevertheless, surface portions may be softened or dissolved during use. In the event that compositions are found which are satisfactorily form-retaining for applications to material to be conditioned, while still being sufficiently plastic under dryer conditions to

avoid cracking, they may not require the presence of the plasticizing agents of this invention for improved effects or may require lesser proportions thereof than other comparable more rigid fabric treating compositions. Normally, however, the fabric conditioning agents are solid state materials which can benefit from the addition of the plasticizers.

Specific examples of surface active materials of the types described above are given in Volume II of the text, *Synthetic Detergents*, by Schwartz, Perry and Berch, published in 1958 by Interscience Publishers, New York. See pages 25 to 143. Among the more preferred of these are:

Nonionic — nonylphenoxy polyethoxy ethanol; stearic monoethanolamide, lauric monoethanolamide, block copolymers of ethylene oxide and propylene oxide (Pluronics ®),

Anionic — sodium soap of mixed coconut oil and tallow fatty acids; sodium stearate; potassium stearate; sodium laurate; tallow alcohols sulfate;

Cationic — dilauryl dimethyl quaternary ammonium chloride; hydrogenated tallow alkyl trimethyl ammonium bromide and benzethonium chloride.

In the recitation of conditioning agents given above, there are included compounds whose utility as conditioning agents in automatic laundry dryer processes such as those described herein were discovered by others. It is to be understood that the present invention is of the incorporation of a plasticizer in such compositions to improve their properties. The invention is generally applicable to all solid state conditioning compositions used in such processes and it is considered unnecessary to recite here the host of conditioning agents that can be improved by this method.

The plasticizers that are used are highly preferably liquids but it may sometimes be desirable to replace part or, in some circumstances, all of the liquid state plasticizer with one which is a solid but has the properties of a liquid or near-liquid in combination with the conditioning agent or mixture of agents employed. Thus, the materials normally known to have plasticizing properties for various solids are useful, providing that under the conditions of the dryer, they sufficiently plasticize or soften the conditioning composition or make it resilient so as to improve its resistance to cracking and flaking.

Of the plasticizing agents it is preferred to use those which are water soluble and liquid at room temperature, or 25° C. Although not as useful to make the best conditioning compositions, plasticizers which are oil or alcohol soluble and which are solids at room temperature may be used in appropriate circumstances. With respect to the solid plasticizers, those which soften or liquefy under the slightly elevated temperatures of initial dryer conditions are best. Of course, the plasticizers should be chosen so that the most desired effects are obtained with the particular compositions employed. For example, an anionic plasticizer would not normally be used with a cationic conditioning agent nor would a near-solid plasticizer be employed with a very rigid solid state conditioning agent. Although by following the guide lines previously given, a wide variety of plasticizing materials may be used to improve the present conditioning agent, normally there will be employed liquid, colorless, water soluble, nonionic materials, generally of comparatively low molecular weight, e.g., from 100 to 1,000, preferably 100 to 500. These will normally be poly-lower alkoxy or polyhydroxy com-

pounds, wherein the lower alkylene oxide or hydroxy groups contribute water solubility and liquid characteristics. Most preferably, the alkoxy groups will be ethoxy, and generally the number present will be from 2 to 20 per molecule. For the polyhydroxy compounds, there will usually be present from 2 to 6 hydroxyls.

Representative of the polyoxyethylene glycol derivatives are the alkyl phenyl polyoxyethylene ethanols wherein there are present 2 to 20 ethoxy groups per molecule. The alkyl may be from 1 to 20 carbon atoms and there may be several alkyl groups on the phenyl ring. Generally, there will be no more than 3 alkyl groups and usually they will be of 6 to 12, preferably from 7 to 9 carbon atoms. The chain length of the polyoxyethylene moiety will normally be chosen to make the compound water soluble. Thus, with a single octyl or nonyl group on the phenyl, there will usually be present from 5 to 10 ethoxy groups on the side chain. Another class of liquid plasticizer is that of the poly-lower alkylene glycol type, preferably polyethylene glycol of 2 to 20 ethoxy groups per molecule. Often, such compounds will have a multiplicity of free hydroxyl groups to give them water solubility. In some instances, poly-lower alkylene glycol may comprise a mixture of ethylene and propylene glycol moieties, either randomly distributed or as blocks, with it being preferred that the proportion of the lower alkylene oxide present should be great enough to impart water solubility. Yet, providing that there is a sufficient balance of hydrophilic groups in the molecule to impart a hydrophilic character to it, compounds of this type in oil form, such as the Ucons ®, may be used if they are hydrophilic enough to be readily distributed over the fabric with the conditioning agent.

Of the polyhydroxy compounds that are useful, the most preferred is glycerol, although propylene glycol, ethylene glycol and similar diols and triols are also good plasticizers. All such materials, including other suitable polyols, are liquids and have hydrophilic properties. In combination with the solid state fabric softeners and antistatic agents, they produce strengthened compositions which are more resistant to strains than the unplasticized conditioning agent. In some circumstances, liquids which do not possess hydrophilic natures are useful and of these the mineral oils, esters, e.g., phthalates, sebacates, ketones and acids are acceptable, usually in very minor proportions, providing that they are readily distributed with the conditioning agent and, in such formulas, do not spot or stain the fabric. The esterified di-carboxylic acids, such as the sebacates, will normally possess substantially terminally located carboxyl groups and intermediate alkylene chains, usually of from 4 to 10 carbon atoms. The esterifying alcohols will generally be of from 3 to 10 carbon atoms. Of these compounds, dibutyl sebacate, dioctyl phthalate and dioctyl sebacate are preferred.

Of course, to be a satisfactory plasticizer, the vapor pressure of the liquid should be low enough so that it will not be lost by evaporation during storage of the treating composition or article. Again, as was mentioned before, solid materials that liquefy at the slightly elevated temperatures of the initial drying period may be used. Among these may be mentioned the fatty acids and alkoxylation fatty acids or hydroxy fatty acids. It has been noted that although some higher fatty acids are not really plasticizers, having melting points that are too high, when they are compounded with various conditioning agents of a more friable type, they contribute to

strengthening of the compositions and thereby help to prevent excessive spotting and staining of treated articles.

In addition to the fabric softening and/or antistatic agents and plasticizers in the present compositions, other components may also be present for their adjuvant effects. Thus, other conditioning agents may be used, including those designed to treat the fabrics in other ways than in softening. For example, perfumes, brighteners, bactericides, solvents, thickening or hardening agents, stabilizers and other materials may be incorporated in the conditioning compositions. In some cases, small quantities of water may be present, especially when the components form hydrates. The types and proportions of such adjuvants used will be chosen to be readily applied with the softening agents and will not interfere with their operation.

The final conditioning composition is preferably waxy in appearance and is capable of being stored at room temperature without melting, while yet being satisfactorily picked up by fabrics in the operation of an automatic laundry dryer, when the fabrics tumble into contact with the conditioning composition. The conditioning composition will be form-retaining at temperatures below 30° C. and preferably, also at all temperatures below 40° C. It may tend to fuse or melt under the higher temperatures obtained in the dryer, such as 70° to 90° C. but usually will be only sufficiently softened, even in the presence of the plasticizers, to be abraded off a treating article onto the surface of material to be conditioned, at dryer conditions, including the presence of moisture and drying gas at an elevated temperature. The conditioning composition should be removable from a substrate at a regular rate and in sufficient quantity to condition fabrics, at a temperature from 40° to 90° C., preferably from 50° to 80° C. Normally, to effect these purposes, the fabric softener and/or antistatic agent, the surface active conditioning agent mentioned previously, will be a major proportion of the conditioning composition, usually from 51 to 99% thereof. Preferably it will comprise from 75 to 95% of the composition. The plasticizer will be from about  $\frac{1}{2}$  or 1 to 25% of the composition, preferably from 5 to 20% thereof. Other adjuvants, such as those previously mentioned, may be present to make up the balance of the composition and usually this will total from 0 to 48%, preferably from 5 to 20% thereof.

When the conditioning composition is employed as a coating on the substrate, the thickness of the coating applied will normally be within the range of 0.0005 to 0.5 centimeter, generally from 0.002 to 0.3 cm. and preferably from 0.003 or 0.01 to 0.1 cm. The thickness given is that external to the outer surface of the object coated. A somewhat porous or rough surfaced object or one having indentations will normally be preferred so that the coating composition may penetrate below the outer surface to a sufficient depth to hold the external coating firmly to the surface and prevent its cracking or flaking off from the surface during use. In addition to the plasticizer helping to prevent cracking and flaking, it also aids in the penetration of the pores or openings in the surface of the substrate and thereby assists in holding the coating to the base. A minor proportion of the external thickness of coating agent may be below the surface. This will usually be held to 10 to 30% of that external to the base. In terms of weights applied, the conditioning composition will normally be employed in the range of 0.0005 to 0.5 g./sq. cm., preferably from

0.002 to 0.3 g./sq.cm. and most preferably from 0.01 to 0.2 /sq. cm., with 0.5 to 15 grams used per 5 to 10 pounds of laundry.

The manufacture of the present compositions is relatively simple. Usually, a melt of the various constituents may be prepared or, if desired, a solvent may be used to dissolve or disperse all of them. The choice will depend upon the method of applying the composition to a substrate. In the event that the composition is employed as a solid or is used later to coat other bases, it may be made by either the fusion or dissolving methods, followed by solidification by cooling or evaporation of solvent. Alternatively, mere physical mixing may be employed. The use of melts and the advantages of these in the coating of substrates are described in the patent application entitled *PROCESS FOR THE MANUFACTURE OF FABRIC CONDITIONING ARTICLE*, filed by me on the same day as the present application. When melts are employed the surface will be cooled soon after application of the desired thickness of conditioning agent. When solutions are used, the solvent contents thereof will normally be from 20 to 80%, preferably from 20 to 40%, and solvent will be evaporated almost immediately after application. It is not necessary to completely dissolve all the constituents of the conditioning composition, so long as they are satisfactorily dispersed. The application of the conditioning composition is made to the desired depth on the base employed in either a single step or plural step application, with solidification of the coating between steps. Penetration of the surface of the base may be regulated by adjusting the composition viscosity or by modifying the nature of the base surface. Preferred methods for coating solids, such as spheres, include spraying and rolling and sphere in a shallow pan of coating composition. When coating flexible items such as paper, roll coating, dip coating, or spray coating may be used. Care will normally be taken to limit the penetration of the depth coating below the surface of the article being coated and to prevent impregnation thereof, inasmuch as the internally located conditioning composition often will not be useful because it cannot be abraded off the conditioning article by the tumbling fabrics contacting it.

The present compositions and articles are simple to employ and the treating methods are effective for conditioning fabrics without special care being necessary on the part of the user. The conditioning article is placed in the automatic dryer or other tumbling device immediately before a drying or treating operation commences. In tumbling, the laundry moves past the conditioning article and the combination of abrading action, heat and moisture causes the deposit of conditioning agent on the fabrics. Although it is preferred to employ an automatic laundry dryer, equivalent machines may be used and in some instances the heat and drying air may be omitted for part or all of the cycle. Generally, air will be employed and will be circulated frequently. Normally there will be about 5 to 50 changes of drying gas in the dryer drum per minute and the gas temperature will be from 10° to 90° C., preferably from 50° to 90° C. The dryer will usually revolve at about 10 to 100 revolutions per minute, preferably 20 to 60 r.p.m. The weight of laundry employed will usually be from 4 to 12 pounds, preferably from 5 to 10 pounds, dry weight. This will fill 10 to 70% of the volume of the dryer, preferably about 30% to 60% thereof. Drying will usually take from 5 minutes to 2 hours and generally from 20 minutes to 1 hour will be sufficient, with synthetic

fabrics, such as nylon, polyesters and synthetic-natural blends requiring shorter periods of time than cotton laundry. The synthetics may often be dried satisfactorily in from 3 to 10 minutes and resin-treated fabrics of the permanently pressed or non-wrinkling types may be dried in from 10 minutes to  $\frac{1}{2}$  hour.

After completion of the drying of the laundry or the softening operation, the conditioning article is removed and examined. If sufficient softener remains, the article may be employed again until complete removal of the coating. If the laundry is not satisfactorily conditioned, additional tumbling may be in order. To obtain different levels of conditioning activity or different effects there may be employed several treating articles or a plurality of different treating articles. Of course, after the coating is consumed the bases may be discarded. Otherwise, additional coatings may be applied to them and the articles can be used again. The coating compositions may be marketed as mixtures, solidified melts or in appropriate solvents, so as to enable the user to recoat the bases, if desired. Other details about the use of the present compositions, articles and methods may be found in an application for patent entitled *FABRIC CONDITIONING METHODS, ARTICLES AND COMPOSITIONS*, filed by G. T. Hewitt, et al. on the same day as the present application, as well as in my other patent application, previously mentioned.

Although the principal advantages of the present invention reside in the avoidance of spotting of the treated fabrics, caused by flaking off of pieces of conditioning composition and subsequent fusing thereof onto the treated fabric, other advantages also result from utilization of this invention. As was mentioned, the plasticizers help the conditioning agent to penetrate better under the surface of the substrate, thereby better holding the coating and preventing flaking, in addition to making the coating itself more resilient and less apt to crack upon subjection to strain or shock. The hydrophilic plasticizers, especially those which are of good water solubility, assist in smoothly removing the conditioning composition from the article and in aiding it to make good contact with the fabric to be treated. Once deposited on the fabric, the plasticizers help to spread it more evenly over the surface. They do this without contributing objectionable properties to the conditioning article or composition. So even if a smear, lump or flake is deposited, the plasticizer helps to distribute it and improves the appearance of the treated fabrics.

The following examples are provided to illustrate the various embodiments of the invention. Unless otherwise indicated, all parts are by weight, temperatures are in degrees Centigrade and the measurements are in the metric system. It should be borne in mind that the examples are only intended to be illustrative of the invention and do not limit its scope. For example, although the particular active ingredients disclosed may be employed best, those which are obvious modifications thereof (chemically different but physically equivalent, as in substituted alkyl phenyl polyoxyethylene ethanols) or otherwise equivalent (other plasticizers), are also within the scope of the invention.

#### EXAMPLE 1

|                                                                                                                 | Parts by weight |
|-----------------------------------------------------------------------------------------------------------------|-----------------|
| Stearic monoethanolamide<br>(from hydrogenated tallow fatty acids)                                              | 90.0            |
| Nonyl phenoxy polyoxyethylene ethanol<br>of 5 oxyethylene groups (Triton N 101,<br>mfd. by Rohm and Haas, Inc.) | 10.0            |

#### EXAMPLE 1-continued

| Parts by weight |
|-----------------|
| 100.0           |

5 A melt of the above composition is prepared and is used to coat a foamed polystyrene sphere having a diameter of 10 cm. The sphere is made by cutting to shape from slabs of polystyrene foam board and has the rough edges thereof rounded off, to prevent snagging with clothing in an automatic laundry dryer treatment. The styrofoam sphere is coated with a melt of the above composition to a depth of 0.05 cm. above the surface of the styrofoam and penetrates to a depth of about 0.01 10 cm. below that surface. The density of the sphere is approximately 0.3 g./c. cm. and the weight of conditioning composition applied to it is about 18 grams. The coating is effected by rolling the sphere evenly in a shallow pan containing the melted coating agent and immediately after application, cooling the coating to solidify it.

15 The conditioning action of the article made is tested by employing it in conditioning a dryer load of 8 pounds of mixed laundry in an automatic laundry dryer. The laundry treated is a mixture of wearing apparel and household articles, including cotton, synthetic fibers, especially polyesters, polyacetates and blends of these plastics with each other or with cotton, nylons, rayons and resin-treated, permanently pressed and wrinkle 20 resistant fabrics. The wash comprises approximately 50% of cotton articles, 20% of polyester-cotton blends, 10% permanently pressed items, 10% nylon articles and the balance of rayon, acetate, etc. The dryer employed is of the horizontal drum type, having longitudinal flights or ridges to assist in creating a tumbling action. After loading the damp laundry, just removed from a washing machine after having been spun "dry", the conditioning sphere, containing a coating of conditioning agent, is placed on top of the laundry, which occupies 25 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 97

with the same coating, nylon articles are removed after 5 minutes and permanently pressed articles are removed after 15 minutes. Even the diminished treatment times employed are effective to make the fabrics antistatic and soft and they are wrinkle-free. When, in such runs, the nonyl phenol polyoxyethylene ethanol constituent is omitted from the fabric treating coating, the coating tends to crack and flake and on occasion, spots the clothing being treated, especially the permanently pressed articles.

When, instead of the formation shown above, there is employed 95% of stearic monoethanolamide and 5% of nonyl phenol polyoxyethylene ethanol, the softening effects are not quite as good as these obtained with the above composition but there is no spotting of laundry apparent, either. The coating in such case does not appear to be as strong or resilient as that described above. Also, when 50% of stearic monoethanolamide and 50% of nonyl phenol polyoxyethylene ethanol are used, softening is appreciably diminished and some spotting is apparent.

Effects corresponding to those mentioned herein are also obtained when the conditioning composition is modified to include other lower alkanolamides of higher fatty acids, and mixtures thereof, anionic softening agents, such as soap or sodium lauryl sulfate, or cationics, such as distearyl dimethyl ammonium chloride. Similarly, the plasticizer may be changed to a lower alkylene or polyalkylene glycol, such as propylene glycol or polyethylene glycol, glycerol, or dibutyl sebacate, to also obtain improved conditioning composition effects. However, for most of the plasticizers, except for esterified sebacates and similar esters, at least 1% of plasticizer should be present and preferably, from 5 to 20% thereof.

## EXAMPLE 2

The procedure of Example 1 are employed, except that the conditioning composition is applied as an alcoholic solution, comprising 30% ethanol, to paper sheeting having a thickness of about 0.005 cm., which is thus impregnated with conditioning composition at the rate of 3 grams thereof per thousand sq. cm. The paper sheets are approximately 20 × 25 cm. and the thickness of conditioning composition below the surfaces thereof is about 0.001 cm.

Despite the fact that the flexible paper is much more readily distortable than is the polystyrene sphere of Example 1, when employed in the dryer under the same conditions as specified in the preceding example, conditioning compositions on the paper are strengthened by the presence of the nonyl phenol polyoxyethylene ethanol or other suitable plasticizer and do not flake off or crack. Thus, no spotting or staining of treated fabrics is noted. When similar products are used, without plasticizer in the conditioning composition, occasionally some of the papers become twisted in such manner as to cause pieces of conditioning composition to be deposited in flakes or sections on fabrics to be treated, creating an objectionable spotting or staining.

As is the case in Example 1, when others of the named conditioning plasticizing materials are employed instead of those of the 90:10 formula of Example 1, including compositions in which proportions are varied as is indicated in that example, similar good conditioning results are obtained, wherein the articles treated are made soft, static-free and wrinkle resistant.

## EXAMPLE 3

|                                                                                | Parts by weight |
|--------------------------------------------------------------------------------|-----------------|
| Sodium soap of a mixture of fatty acids<br>(75% tallow, 25% coconut oil acids) | 15.0            |
| Stearic monoethanolamide                                                       | 84.5            |
| Diocetyl sebacate                                                              | 0.5             |

The above composition is melted and applied to both polystyrene foam spheres and 20 cm. × 25 cm. papers, as a melt, producing coatings about 0.002 cm. thick on the base papers and about 0.1 cm. thick in the case of the spheres. Penetration is about 25% of the exterior layer of conditioning composition.

When used to treat laundry in the manner described in Example 1, the products are non-flaking and do not spot the laundry. Yet, they condition it very satisfactorily, making it soft and static-free. When the amount of diocetyl sebacate is increased or when it is replaced by other dialkyl polybasic alkanoic acids, similar good results are obtained. Such results also obtain when various other combinations of the previously mentioned conditioning agents and plasticizers are employed. Of course, efforts will usually be made to find the most desirable compositions, which condition best and do not spot materials being treated.

## EXAMPLE 4

78% of stearic monoethanolamide, 10% of nonyl phenol polyoxyethylene ethanol and 12% of a 50-50 coco-tallow sodium soap are employed, either as a melt or in alcoholic solution, to treat form-retaining and flexible bases. Excellent softening is obtained with no staining at all under the conditions described in Example 1. Of course when other dryer conditions are employed, providing that the drying gas temperature is within the range of from 40° to 90° C., preferably from 50° to 80° C., and the tumbling time if from 3 minutes to 2 hours, good conditioning and no spotting or staining is also experienced.

What is claimed is:

1. An article for conditioning fibrous materials by treating them with a conditioning composition which comprises a solid base, at least one side of said base coated with a continuous coating of a conditioning composition comprising a major proportion of non-ionic, anionic or cationic surface active conditioning agent and from 1 to 25% by weight of conditioning composition of plasticizing agent selected from the group consisting of water soluble alkyl phenyl polyoxyethylene ethanols containing from 2 to 20 oxyethylene groups, the alkyl containing from 6 to 12 carbon atoms, water-soluble poly-(C<sub>2</sub> - C<sub>3</sub>) - alkylene glycols having from 2 to 20 C<sub>2</sub> - C<sub>3</sub> alkoxy groups per molecule, lower alkyl polyols of 2 to 6 hydroxy groups per molecule and esterified dicarboxylic acid containing substantially terminally located carboxyl groups and an intermediate alkylene chain of from 4 to 10 carbon atoms, said acid being esterified with C<sub>3</sub> - C<sub>10</sub> alcohol and wherein from 10 to 30% of the thickness of said composition penetrates said base said plasticizing agent improving the transferability of the conditioning agent to the fibrous materials by preventing cracking or flaking off of conditioning agent from the base during a conditioning operation in which the conditioning article is in control with tumbling fibrous materials for a time long enough to apply a sufficient amount of conditioning composition to such materials to condition them.
2. An article according to claim 1 wherein the conditioning composition comprises a fabric softening or antistatic agent and the plasticizing agent is a liquid at 25° C.

\* \* \* \* \*